

# UNITED STATES PATENT OFFICE.

CAMILLE CLERC, OF PARIS, FRANCE, ASSIGNOR OF ONE-HALF TO ARMAND NIHOUL,  
OF PARIS, FRANCE.

## PROCESS FOR EXTRACTING TIN FROM TIN-PLATE CHIPS.

1,413,555.

Specification of Letters Patent. Patented Apr. 18, 1922.

No Drawing.

Application filed January 26, 1922. Serial No. 532,010.

*To all whom it may concern:*

Be it known that I, CAMILLE CLERC, a citizen of France, and a resident of Paris, France, have invented new and useful Improvements in Processes for Extracting Tin from Tin-Plate Chips, which is fully set forth in the following specification.

Heretofore tin has been extracted from tin-plate chips or shavings (or scraps) through action thereon of chlorides of tin and of iron, but in the usual process the dissolution of tin in these chlorids is seldom complete. The same is particularly insufficient when tin-plate chips are treated in this way to allow the sheet-iron deprived from tin to be used for making steel, because tin-spots remain on the iron.

According to the present invention, these difficulties are obviated by the fact that a vacuum is produced in the receptacle containing the tin-plate chips, during the dissolution of tin by means of perchlorides of tin or iron. The said vacuum facilitates the escape of the gases produced and allows the reaction to be fully carried out.

The tinny matters are put in a tight-closure container to which a solution of perchloride of tin or iron is added, so that the matters to be treated are entirely immersed in the same. The vacuum is then created

and increased as far as it is practically possible, for instance up to about a 15 or 20 cm. mercury column.

According to the process forming the subject-matter of the invention, the tin is quickly dissolved while the perchlorides are converted into protochlorides of tin or iron. These protochlorides of tin or iron are then treated in the usual way. The tin extracted therefrom by dissolution is precipitated by zinc, iron or any other suitable agent. The solution can also be treated again by the addition of chlorine for instance, so that the initial solutions of iron or tin chlorides can be reobtained.

While I have specified perchloride of tin in the claim, it is to be understood that I consider perchloride of iron as a full equivalent for the purpose of this invention.

What I claim is:

Process for extracting tin from scrap tin-plate and the like, consisting in subjecting said tin-scrap to the action of perchloride of tin in a closed receptacle while maintaining therein a vacuum to facilitate the reaction, and treating the resulting solution with a metal to precipitate the tin.

In testimony whereof I have signed this specification.

CAMILLE CLERC.